

1

3,498,855

## AMMONIUM NITRATE PROPELLANT COMPOSITIONS CONTAINING THERMOPLASTIC POLYMERIC RESINS

Samuel W. Harris, Chicago, Ill., assignor to Standard Oil Company, Chicago, Ill., a corporation of Indiana  
No Drawing. Filed July 24, 1967, Ser. No. 655,300  
Int. Cl. C06d 1/00

U.S. Cl. 144—19

5 Claims

### ABSTRACT OF THE DISCLOSURE

Novel propellant compositions comprising ammonium nitrate as a primary oxidizer and thermoplastic polymeric resins having ionic and covalent bonds, as the binder.

### BACKGROUND OF THE INVENTION

This invention relates to a new class of propellant compositions and more particularly to ammonium nitrate compositions having improved ballistic properties, as a result of a novel binder system.

The use of ammonium nitrate-based compositions as a solid propellant is attractive because of the cheapness and availability of ammonium nitrate, because of the relatively low flame temperature of decomposition of ammonium nitrate, and because the excess free oxygen available from the decomposition permits the use of oxidizable material to improve the energy available from the decomposition. However, the physical characteristics of ammonium nitrate and grain material produced therefrom introduced problems with respect to choice of binder material. Solid ammonium nitrate exists in different crystalline forms at different temperatures and the transition from one form to a different form involves a volume change of the ammonium nitrate. Volume changes which occur at about 90° F. and also at about 0° F. are particularly destructive to shaped propellant grains. It is, therefore, obvious that ammonium nitrate-based compositions could be seriously affected by storage at temperatures common to such storage conditions.

One requirement for solid propellants suitable for military use is that the propellant be ballistically stable after long periods of storage at temperatures as high as 160° F. and as low as —65° F. Another requirement is that the grain composition not shatter or crack after being subjected to alternate high and low temperatures (i.e. cycled from the high temperature immediately to the low temperature at least twice); and that the burning of the composition following such cycling be uniform and not changed materially from the burning characteristics of such grain material which has not been subjected to such cycling. The binder material used with the ammonium nitrate to form physically stable grains must be flexible enough to compensate for changes in volume of the ammonium nitrate as it passes from one temperature to another, in order that such changes produce a minimum amount of voids and cracks in the grain. Production of fissures in the grain either internally or externally of the surface of the grain creates additional burning surface which results in unpredictability of the ballistic performance of the grain. Furthermore, the binder material must be of such nature to permit grain formation by methods known to the art, i.e. extrusion, molding, etc.

### SUMMARY OF THE INVENTION

I have now discovered a novel propellant composition comprising ammonium nitrate as the oxidizer and a thermoplastic resin having ionic and covalent bonds, as the binder. The oxidizer and binder must be in intimate

2

physical mixture. The present compositions may also contain various other additives such as catalyst for the promotion of combustion, carbon, chemical stabilizer, etc.

The term "ammonium nitrate" as used in this specification and in the claims is intended to mean either ordinary commercial grade ammonium nitrate such as conventionally grained ammonium nitrate containing a small amount of impurities which may be coated with a small amount of moisture-resisting material such as petrolatum or paraffin, or to mean military grade ammonium nitrate or mixture of minor amounts (usually less than 10%) of other organic or inorganic nitrates such as, guanidine nitrate or sodium nitrate or potassium nitrate with the ammonium nitrate. A mixture of finely ground and unground or coarsely ground ammonium nitrate is preferred. The major proportion of the ammonium nitrate should be finely ground in order to reduce the voids to a minimum and hence avoid the use of excess binder material. It is well known in the propellant art that particle size and size distribution within the composition are related to the ballistic properties. The amount of grinding then, will depend upon the desired properties of the propellant.

The polymeric binder material is a cross-linked thermoplastic resin linked by ionic and covalent bonds, characterized by strong interchain forces. These interchain forces are developed between ionized carboxyl groups pendant from an alpha olefin chain and metallic ions selected from the group consisting of sodium, potassium, calcium, magnesium and zinc. These products may be obtained commercially from E. I. du Pont de Nemours and Company under the name "Surlyn A." The major constituent of "Surlyn A" is ethylene. The polymeric binder has a softening point in the range of 80 to 120° C., and a preferred softening point of 90 to 105° C. These new propellant compositions have the advantage of excellent ballistic properties, simplicity of formulation and stability. Normal mixing of the composition is accomplished without the necessity of additional plasticizers. The present compositions provide a propellant which may be utilized where a low burn rate is required.

It is desirable that catalyst be present in the composition and any catalyst known to be effective for the combustion of ammonium nitrate grains containing oxidizable thermoplastic binder materials may be used. These include certain iron compounds broadly designed as Prussian Blues, sodium barbiturate, etc. Catalysts which are exceptionally suitable to the present compositions are disclosed in copending application, S.N. 655,328, filed July 24, 1967. These compositions comprise hydrocarbons which readily form peroxides.

It is also desired that the composition contain a carbon component. The finely divided carbon may be added in amounts up to 10% by weight of the composition, preferably in amounts of 1 to 5% by weight for the purpose of improving ignition and the burning rate of the composition. Highly adsorptive activated carbons such as "Norite" and "Nuchar" well known in the art as activated carbon of vegetable origin, make up one class of effective burning rate components. A second general class of carbon useful for increasing the burning rate of compositions are the carbon blacks, roughly classified as the channel blacks and the furnace combustion blacks. The carbon blacks are characterized by low ash content, that is, less than about 0.5%, usually less than about 0.15%, and by having extremely small particle size, that is 50 to 5,000 Å. and contain adsorbed hydrogen and oxygen. "Bead" type carbon blacks, such as Micronex Beads and Statex Beads, are also suitable. A third type of carbon which may be used is finely ground petroleum

coke, particularly petroleum coke obtained as residue in the pipe-stilling of mid-continent heavy residuums.

The oxidizer and binder should be present in the composition in essentially stoichiometric amounts, in order to best utilize the excess oxygen obtained from the oxidizer. Therefore, a major amount of oxidizer and a minor amount of binder should be present. Suitable propellant compositions comprise:

|                                                            | Percent by weight |
|------------------------------------------------------------|-------------------|
| (a) Binder                                                 | 5 to 40           |
| (b) Catalyst                                               | 0.5 to 5          |
| (c) Carbon                                                 | 0 to 10           |
| (d) Remainder of composition essentially ammonium nitrate. |                   |

Preferred compositions are as follows:

|                                                            | Percent by weight |
|------------------------------------------------------------|-------------------|
| (a) Binder                                                 | 15 to 30          |
| (b) Catalyst                                               | 1.5 to 3.5        |
| (c) Carbon                                                 | 1 to 5            |
| (d) Remainder of composition essentially ammonium nitrate. |                   |

Other additives which may be added are present in an amount sufficient to provide effective improvement of the properties for which they are added.

In preparing the composition of this invention, any procedure known to the art for the separation of ammonium nitrate grains containing a thermoplastic binder may be used.

With respect to the properties of a solid propellant, the velocity at which a solid propellant is consumed during operation is called the burning rate. It is measured in a direction normal to the propellant surface and is usually expressed in inches per second. The burning rate may be expressed by the following relation, in which the influence of all performance parameters is small compared to the chamber pressure and the initial grain temperature.

$$r = ap_e^n$$

The burning rate or velocity of propellant consumption "r" is usually given in inches per second; the chamber pressure "p<sub>c</sub>" in pounds per square inch; "a" and "n" are constants. The constant "a" varies with the initial propellant temperature, and thus the burning rate is a function of the temperature of the grain prior to combustion. The lower the value of "n," the less is the detonating character of the decomposition of a gas producing composition and the more even and smooth is the burning rate of the propellant grain. Thus, a sustained thrust rather than a detonation is obtained by smooth burning of the grain.

The temperature sensitivity for different solid propellants is usually expressed as the percentage change of thrust per unit of temperature change. Temperature changes effect the equilibrium pressure and the burning rate. The definitions of the temperature coefficients are given by Sutton, "Rocket Propulsion Elements" (2nd ed. 1958).

$$\pi_K = \left( \frac{\delta \ln p}{T} \right)_K = \frac{1}{P_e} \left( \frac{\delta P}{\delta T} \right)_K$$

$$\sigma_p = \left( \frac{\delta \ln r}{\delta T} \right)_p = \frac{1}{r} \left( \frac{\delta r}{\delta T} \right)_p$$

Here  $\pi_K$  is the temperature sensitivity coefficient of equilibrium pressure at a particular value of K (K is the ratio of the burning surface to the throat area), expressed in percent pressure change per degree temperature change. Mathematically it is defined as the partial derivative of the natural logarithm of the equilibrium chamber pressure  $p$  with respect to temperature  $T$ . The other temperature sensitivity coefficient  $\sigma_p$  refers to the change in burning rate  $r$  of a solid propellant with respect to temperature  $T$  at a particular value of chamber pressure  $p_c$ . It is also known as the burning rate temperature coefficient.

efficient, while  $\pi_K$  is known as the temperature sensitivity of pressure.

For most propellant applications, as low a temperature coefficient as possible is desirable and even required for engineering design consideration. Lower pressure levels over a given temperature level allows a sizable weight savings for most missile applications.

#### DESCRIPTION OF PREFERRED EMBODIMENTS

The following examples are given by way of illustration and should not be construed as limiting.

#### EXAMPLES I-VII

The following procedure was used in producing the propellant grains identified in the examples:

The pre-ground ingredients were mixed in a sigma blade mixer using a 110° C. jacket temperature, until the mixture was a plastic mass.

All the compositions shown below contain Surlyn A binder (identified as "binder" in the examples) having a softening point of about 95° C., and contained sodium as the primary metallic ion. The compositions are as follows:

| Example | Formulation                                            | Weight Percent             | Catalyst Type        |
|---------|--------------------------------------------------------|----------------------------|----------------------|
| 25 I    | Ammonium nitrate<br>Carbon black<br>Binder<br>Catalyst | 78.0<br>3.0<br>17.0<br>2.0 | Octahydroanthracene. |
| II      | Ammonium nitrate<br>Carbon black<br>Binder<br>Catalyst | 78.0<br>3.0<br>17.0<br>2.0 | Phenylecumene.       |
| 30 III  | Ammonium nitrate<br>Carbon black<br>Binder<br>Catalyst | 73.0<br>5.0<br>20.0<br>2.0 | Silica-alumina.      |
| IV      | Ammonium nitrate<br>Carbon black<br>Binder<br>Catalyst | 73.0<br>5.0<br>20.0<br>2.0 | Tetralin and cumene. |
| 35 V    | Ammonium nitrate<br>Carbon black<br>Binder<br>Catalyst | 78.0<br>3.0<br>17.0<br>2.0 | Tetralin.            |
| VI      | Ammonium nitrate<br>Carbon black<br>Binder<br>Catalyst | 78.0<br>3.0<br>17.0<br>2.0 | Cumene.              |
| 40 VII  | Ammonium nitrate<br>Carbon black<br>Binder<br>Catalyst | 78.0<br>3.0<br>17.0<br>2.0 | Asphalt.             |

The above formulations were molded into grains and cut into strands for testing in a Crawford bomb. The results of the tests are shown in Table I.

TABLE I

| Product of Example | Ballistic Properties |            |         |                       |
|--------------------|----------------------|------------|---------|-----------------------|
|                    | n                    | $\sigma_p$ | $\pi_K$ | $r_{1000}$ (in./sec.) |
| I                  | 0.55                 | 0.112      | 0.25    | 0.044                 |
| II                 | 0.34                 | 0.112      | 0.17    | 0.034                 |
| III                | 0.63                 | 0.28       | 0.77    | 0.036                 |
| IV                 | 0.45                 | 0.135      | 0.25    | 0.031                 |
| V                  | 0.75                 | 0.0826     | 0.33    | 0.034                 |
| VI                 | 0.64                 | 0.172      | 0.48    | 0.038                 |
| VII                | 0.68                 | 0.155      | 0.48    | 0.036                 |

Table I clearly shows excellent ballistic properties afforded by the present composition.

What is claimed is:

1. A propellant composition comprising:
  - a major amount of ammonium nitrate in intimate physical mixture with;
  - a polymeric binder material, having a softening point in the range of from 80° C. to 120° C., said binder material comprising a cross-linked thermoplastic resin containing:
    - i) a major amount of ethylene units; and
    - ii) interchain forces developed between carboxyl groups pendant from an alpha olefin chain and metallic ions selected from the group consisting of sodium, potassium, calcium, magnesium, and zinc; and

- (c) an effective amount of combustion catalyst.
2. The composition of claim 1 wherein said polymeric binder material is present in an amount from 5 to 40 weight percent; said catalyst is present in an amount from 0.5 to 5 weight percent; carbon is present in an amount from 0 to 10 weight percent; and the remainder of said composition is essentially ammonium nitrate.
3. The composition of claim 2 wherein said polymeric binder material is present in an amount of from 15 to 30 weight percent; said catalyst is present in an amount of from 1.5 to 3.5 weight percent; said carbon is present in an amount of from 1 to 5 percent; and the remainder of said composition is essentially ammonium nitrate.
4. The composition of claim 1 wherein said polymeric

5 binded material has a softening point in the range of from 90° C. to 105° C.

- 10 5. The composition of claim 4 wherein said softening point is about 95° C.

#### References Cited

##### UNITED STATES PATENTS

|           |        |                    |          |
|-----------|--------|--------------------|----------|
| 3,147,161 | 9/1964 | Abere et al. ----- | 149—19   |
| 3,305,523 | 2/1967 | Burnside -----     | 149—19 X |
| 3,338,764 | 8/1967 | Evans -----        | 149—19   |

BENJAMIN R. PADGETT, Primary Examiner

U.S. Cl. X.R.

149—20